

## UNITED STATES PATENT OFFICE

2,124,255

## PROCESS FOR THE PRODUCTION OF CORE-ELECTRODES

Franz Leitner, Kapfenberg, Austria

No Drawing. Application May 22, 1935, Serial No. 22,917. In Germany May 23, 1934

2 Claims. (Cl. 219—8)

Core-electrodes having alkaline-earth metals as calcium, magnesium, or the carbides thereof, aluminium or alkaline metals are known.

The use of the aforesaid materials for core wires is limited, however, and requires special working processes. If the core materials have a low melting point, difficulties arise insofar as the core partly or entirely melts when the ingots or billets are heated to a rolling temperature. Thus, if a wire is produced with such materials an irregular form of the core and very often a non-uniform mixture of the different components results. These irregularities cause an irregular melting process and give poor qualities to the deposited metal.

Generally, many core materials alter their chemical composition at the rolling temperature under the influence of heat or of the furnace gases or of the atmosphere. In this way the irregularities of the welding process and poor qualities of the weld are increased.

The present invention consists in selecting only such materials which melt at a higher temperature than about 900° C. and which are chemically stable at this temperature. The selection must be done in such a way that the arc-stabilizing-effect and other requirements for welding are present. The following additional materials are proposed: alkaline earth and/or alkaline compounds containing oxygen and alkaline earth and/or alkaline compounds free of oxygen. Furthermore, metal oxides or compounds of metal oxides and metal alloys in combination with themselves or with the aforementioned materials may be used. The choice should be made in such a way that the above named physical and chemical requirements are fulfilled.

To avoid any detrimental effects of the melting temperature upon the core materials, it is, as a rule, preferred to fill the ingots after casting.

The process may, however, be performed in different ways and some of these are now described. The ingot or billet to be rolled into wire can be made hollow and then provided with additions which are stable at high temperatures. The hole of the ingot or billet can be made by boring, by piercing or by casting the steel around an empty

pipe. The latter pipe, preferably closed at one end, can be made of mild iron or alloy steel of such a composition that its alloying elements have a beneficial influence upon the deposited metal.

An enrichment of alloying metals in the interior of the wire, as a consequence of the use of an alloyed steel pipe has particular advantages. The requirements for a good weld obtained by this process are better than if the metals were equally distributed throughout the whole section. The explanation is that during the welding the atmosphere affects the outer parts of the drops of metal first so that the inner parts containing the alloying elements remain unaffected.

The hollow ingots thus made are afterwards filled with the core materials and worked down to wire.

Another way of carrying out the process consists in inserting the pipe, closed at one end, into the mould filled with the liquid steel and inserting the core materials in the hollow ingot afterwards. It is, furthermore, possible to put a refractory bar containing the additions or an empty steel pipe or a refractory pipe filled with the additions into the pipe before casting and then rolling the ingots. The refractory filling may, if desired, be provided with metallic inserts to make it stronger.

By the last named process, a detrimental effect of the high temperature is hardly to be avoided for which reason, the core materials must be more resistant to heat than if they are filled after casting.

What I claim is:

1. A process for production of core electrodes comprising placing a pipe in a mold containing liquid steel and then filling the pipe with a refractory material having a melting point above 900° C.

2. A process as claimed in claim 1 wherein the refractory material comprises at least one material selected from a group consisting of alkaline earth and alkaline compounds containing oxygen and alkaline earth and alkaline compounds free from oxygen and metal oxides and metal oxide compounds.

FRANZ LEITNER.